

**1**

3,746,628

**METHOD FOR BORIDE COATING STEEL  
ELECTROLYTICALLY**

Wesley G. Kannenberg and William E. Pruden, Endwell, N.Y., assignors to International Business Machines Corporation, Armonk, N.Y.  
No Drawing. Filed Oct. 21, 1971, Ser. No. 191,516  
Int. Cl. C23b 5/00

U.S. CL. 204—39

6 Claims

**ABSTRACT OF THE DISCLOSURE**

A method for improving the formation of a boride coating on steel by utilizing a higher temperature and a higher current density than heretofore whereby a faster diffusion rate is obtained and porosity eliminated.

**BACKGROUND OF THE INVENTION**

The formation of a wear resistant coating on a metal composition and in particular a boride coating on steel is known in the prior art and is described in detail in U.S. Pat. 3,024,176. In the process described in this patent, boride coatings are formed on specific metals by immersing the selected metal and boron in a fused bath composed essentially of at least one alkali metal fluoride and at least one alkali metal fluoroborate so that at least a portion of the bath isolates the metal from the boron. The combination forms an electric cell in which an electric current is generated when an electrical connection, which is external to the fused bath, is made between the metal and the boron. Under such conditions, the boron dissolves in the fused bath and boron ions are discharged at the surface of the metal where they form a deposit of boron which immediately diffuses into and reacts with the metal to form a boride coating. The rate of dissolution and deposition of the boron is self-regulating so that the boron is never deposited at a rate faster than it diffuses and alloys with the metal. If a slower rate is desired, it can be easily controlled by means well known in the art, such as by the amount of resistance in the circuit, surface area exposed to the bath, etc. A limited amount of voltage may be impressed upon the electrical circuit to supply additional direct current if a faster rate is desired.

In the aforementioned patent, it is recommended that in order to produce a reasonably fast plating rate and to insure the fusion of the boron into the metal, the process should be operated in the range of 600° C. to 800° C. It is further recommended that the total current density should not exceed 3 amperes per square decimeter and preferably should not exceed 1 ampere per square decimeter after the boride layer is 1 mil thick. The reason given is that current densities in excess of these ranges lead to some formation of elemental boron in either the form of non-adherent deposits or as granular or large crystalline deposits which give a rough undesirable coating.

It is known that porosity in borided coatings presented a technical problem. Heretofore, porosity has been controlled by keeping the boriding temperature down to 800° C. When boriding was carried out at 900° C., gross porosity developed in the outer portion of the borided coating. Since it would be desirable to operate at 900° C. and above to take advantage of the faster diffusion rates at these temperatures, the problem at hand was to eliminate porosity at these higher temperatures.

**SUMMARY OF THE INVENTION**

In experimenting with the problem of porosity, it was found that porosity occurred at 900° C. because boron diffused inward by a vacancy mechanism leaving a net flux of vacancies moving toward the surface. Coalescence

**2**

of vacancies formed pores at 15 to 25 microns from the surface. It was further found that by using a current density of 8 amperes per square decimeter, much higher than has heretofore been used, a high concentration of boron was maintained at the surface. The high concentration of boron at the surface created a more rapid diffusion of boron that resulted in vacancies being cancelled before they coalesced to form voids.

The ability to produce pore free coatings at temperatures of 900° C. and above permits one to take advantage of the faster diffusion rates at these temperatures. Faster diffusion rates allow deeper coatings to be applied in shorter periods of time. In addition, pore free coatings have a longer wear life that results in savings over coatings containing porosity.

It is, then, a primary object of the present invention to provide a novel and improved method for producing pore free boride coatings.

A further object of the present invention is to provide a novel and improved method for producing a pore free diffusion coating of boron on a metallic substrate at a faster diffusion rate.

A still further object of the present invention is to provide a novel and improved method for producing a pore free diffusion coating of boron on a metallic substrate which utilizes a temperature of at least 900° C. and a current density of at least 8 amperes per square decimeter whereby a faster diffusion rate is obtained.

The foregoing and other objects, features and advantages of the invention will be apparent from the following more particular description of a preferred embodiment of the invention.

**DESCRIPTION OF A PREFERRED EMBODIMENT**

Boriding is accomplished by electrolytic deposition of boron onto the workpiece in a molten fluoride salt bath. In the electrolytic cell, boron chunks in a copper mesh basket act as the anode and the workpiece is the cathode. When an electrical potential is applied to the cell, boron plates out on the cathode. The molten fluoride electrolyte operates between 800° C. and 1100° C. so that the plated boron diffuses into the workpiece. If the workpiece is a low carbon steel, two borides of iron form as FeB on the surface and Fe<sub>2</sub>B beneath it. The hardness of the borides is 1800 Knoop and higher making them suitable as wear surfaces in sliding friction.

The formation of a borided coating takes place in two steps: (1) boron is plated out on the workpiece and (2) boron diffuses into the workpiece to form the intermetallic compounds FeB and Fe<sub>2</sub>B. In order to determine the mechanism of pore formation, the first fundamental question to be answered was whether porosity occurred as a result of the plating process or whether it was a diffusion phenomenon.

The approach taken was to see if porosity could be developed independent of the plating process. If this could be done, porosity would unquestionably be a diffusion related phenomenon. The experimentation was done with a piece of AISI 1020 steel borided at 800° C. with a pore free coating. The sample was copper plated .002"-.003" and given a diffusion anneal at 950° C. for four hours in a nitroreal atmosphere. The FeB layer was eliminated by diffusion of boron into the Fe<sub>2</sub>B layer and the Fe<sub>2</sub>B layer increased in depth. The most important observation, however, was that porosity developed when diffusion took place at 950° C. and it was not present when the sample was originally borided at 800° C. Thus, porosity was developed in a previously pore-free boride coating by allowing diffusion to take place above 900° C. Since this porosity developed in a diffusion anneal, independent of the plating process, porosity was clearly identified as a diffusion phenomenon.

Having established that porosity was related to a diffusion phenomenon, two mechanisms of pore formation were hypothesized. First, a defect structure developed as a means of accommodating a boron concentration gradient in the stoichiometric compounds FeB and Fe<sub>2</sub>B which have no homogeneity range. The second hypothesis was that boron diffused on the boron sub-lattice by a vacancy mechanism in both the FeB and Fe<sub>2</sub>B phases with no diffusion of iron taking place. This created a flux of vacancies moving toward the surface which coalesced to form porosity.

Taking the first hypothesis, it was noted that the phase diagram for the iron-boron system showed that both FeB and Fe<sub>2</sub>B have no homogeneity range. They were depicted by a single vertical line at 33 atomic percent boron and at 50 atomic percent boron. If diffusion was driven by a boron concentration gradient, this gradient may have been accommodated by a defect structure consisting of vacancies, in excess of the equilibrium concentration of vacancies, at the low boron side of the phase boundary between FeB and Fe<sub>2</sub>B. This situation would be analogous to the formation of vacancies on the aluminum rich side of the stoichiometric compound NiAl.

To determine if a boron concentration gradient existed in the stoichiometric compounds FeB and Fe<sub>2</sub>B, electron microprobe traces were run on borided AISI 1020 steel. Traces were obtained by driving the sample across a stationary beam at 4 microns per minute. A chart was run at 0.5 inch per minute so that 10 small divisions on the chart represented 8 microns. The traces showed two plateaus of boron, one in the FeB region and another in the Fe<sub>2</sub>B region. The boron concentration in both the FeB and Fe<sub>2</sub>B phases appeared to be level with no concentration gradient present. In the absence of a boron concentration gradient, abrupt changes in boron concentration occurred at the phase boundaries. There being no boron concentration gradient in either the FeB or Fe<sub>2</sub>B phases, the hypothesis that defect structures occurred by accommodation of a concentration gradient in a stoichiometric compound was rejected.

The second hypothesis stated that boron diffused on the boron sub-lattice by means of a vacancy mechanism in both the FeB and Fe<sub>2</sub>B phases with no diffusion of iron taking place. Iron simply expanded from its bcc or fcc lattice, depending on boriding temperature and carbon content, to the body centered tetragonal lattice of Fe<sub>2</sub>B when the boron concentration reached 33 atomic percent and to the orthorhombic lattice of FeB when the boron concentration reached 50 atomic percent. When boron diffused inward by a vacancy mechanism and no diffusion of iron took place, it created a flux of vacancies moving toward the surface. Vacancies coalesced to form voids which showed up as gross porosity under metallographic examination. Implicit in this hypothesis was the proposition that porosity could be eliminated by increasing the diffusion rate of boron near the surface so that the vacancies moving toward the surface would be cancelled before they coalesced to form voids and porosity. Increasing the diffusion rate of boron near the surface could be accomplished by increasing the concentration of boron at the surface by means of a higher current density.

In carrying out the boriding process with a higher current density, General Electric metalliding equipment was used which comprised essentially an Inconel vessel fitted with a Monel liner. Into the vessel was placed a molten fluoride electrolyte having a composition of 39.3 weight percent LiF, 28.8 weight percent NaF and 31.9 weight percent KF. The vessel was covered with a cover plate which contained two ports for electrodes and one port for a thermocouple well and one port for connection to a bubbler tube. Two glass towers are fitted over the electrode ports with connections to a vacuum source and/or a protective gas atmosphere. A copper mesh basket containing chunks of boron was anode bound by copper wire to a tungsten rod sealed at the top of one electrode tower

with rubber tubing. A similar arrangement was used for a 1" x 1" x .040" strip of AISI 1010 low carbon steel cathode in the other electrode tower.

The vessel was heated by electrical resistance and brought to a temperature of 900° C. under a forming gas (90% nitrogen, 10% hydrogen) atmosphere. A current from a constant current power supply was impressed on the electrolytic circuit by way of an external electrical circuit connecting the anode and the cathode to maintain a current density of 8 amperes per square decimeter on the cathode. The steel strip was immersed half way into the bath and was borided for 4 hours at the constant current density of 8 amperes per square decimeter. An ammeter and voltmeter were connected in the normal way in the external circuit. The pertinent data was:

| Time, min. | Temp., °C. | Current                        |      | Voltage, volts |
|------------|------------|--------------------------------|------|----------------|
|            |            | Density, amps/dm. <sup>2</sup> | Amps |                |
| 0          | 900        | 0                              | 0    | -.20           |
| 1          | 900        | 8.0                            | .96  | +.84           |
| 60         | 900        | 8.0                            | .96  | +.99           |
| 120        | 900        | 8.0                            | .96  | +.10           |
| 180        | 900        | 8.0                            | .96  | +.21           |
| 240        | 900        | 8.0                            | .96  | +.28           |

After the desired time duration of the run is completed, the circuit is turned off, the workpiece is lifted out of the molten salt bath and cooled under forming gas atmosphere in the electrode tower.

A photomicrograph for the above run showed a deep, dense, pore-free coating having a thickness of 5 mils. Similar runs were made at 900° C. using current densities of 2.5 and 4.0 amperes per square decimeter and in both cases the resulting coating was shallow and porous. The series of samples showed that as current density increases the depth of coating also increases when the time and temperature are held constant. The ability to produce deeper coatings is an additional benefit that occurs when the current density is raised to 8 amperes per square decimeter to eliminate porosity.

The high current density produced a lot of fine particles of elemental boron on the surface of the workpiece as expected. The boron particles were interspersed with the fluoride salts and were easily removed with a treatment in boiling water after removal of the workpiece from the electrolytic equipment. The resulting surface was smooth and the boride coating was adherent and pore free.

While the invention has been particularly shown and described with reference to a preferred embodiment thereof, it will be understood by those skilled in the art that various changes in form and details may be made therein without departing from the spirit and scope of the invention.

What is claimed is:

1. A method of forming a boride coating on a low carbon steel workpiece which comprises; forming an electric cell containing a molten fluoride electrolyte composed essentially of lithium fluoride, sodium fluoride and potassium fluoride and having said steel workpiece as the cathode joined through an external electrical circuit to a boron anode; maintaining said electrolyte at a temperature of at least 900° C. in the absence of oxygen; maintaining a current flowing in said electric cell so that the current density at the cathode will not be less than 8 amperes per square decimeter during the formation of the boride coating; and stopping said current flow after a desired time duration of boriding is completed whereby a pore free boride coating of a desired depth is obtained in a shorter time by using a high current density.

2. A method of forming a boride coating on a low carbon steel workpiece which comprises:  
 forming an electric cell containing a molten fluoride electrolyte composed essentially of 39.3 weight percent lithium fluoride, 28.8 weight percent sodium fluoride and 31.9 weight percent potassium fluoride and having said steel workpiece as the cathode joined through an external electrical circuit to a boron anode; 5  
 maintaining said electrolyte at a temperature of at least 900° C. in the absence of oxygen; 10  
 maintaining a current flowing in said electric cell so that the current density at the cathode will not be less than 8 amperes per square decimeter during the formation of the boride coating; and  
 stopping said current flow after a desired time duration of boriding is completed whereby a pore free boride coating of a desired depth is obtained in a shorter time by using a high current density. 15
3. A method of forming a boride coating on a low carbon steel workpiece which comprises:  
 forming an electric cell containing a molten fluoride electrolyte composed essentially of 39.3 weight percent lithium fluoride, 28.8 weight percent sodium fluoride and 31.9 weight percent potassium fluoride and having said steel workpiece as the cathode joined through an external electrical circuit to a boron anode; 20  
 maintaining said electrolyte at a temperature of 900° C. in the absence of oxygen; 25  
 maintaining a constant current flowing in said electric cell so that the current density at the cathode will be 8 amperes per square decimeter during the formation of the boride coating; and  
 stopping said current flow after a desired time duration of boriding is completed. 30
4. The method of claim 3 wherein said current flow is stopped at the completion of 4 hours of boriding whereby a pore free boride coating of a desired depth is obtained in a shorter time by using a high current density. 40
5. A method of forming a boride coating on a low carbon steel workpiece which comprises:  
 forming an electric cell containing a molten fluoride electrolyte composed essentially of 39.3 weight per-

- cent lithium fluoride, 28.8 weight percent sodium fluoride and 31.9 weight percent potassium fluoride and having said steel workpiece as the cathode joined through an external electrical circuit to a boron anode; 5  
 maintaining said electrolyte at a temperature of 900° C. in the absence of oxygen; 10  
 maintaining a constant current flowing in said electric cell so that the current density at the cathode will be 8 amperes per square decimeter during the formation of the boride coating; and  
 stopping said current flow after 4 hours of boriding is completed; and  
 removing the workpiece from the cell and treating it in boiling water to remove boron particles and fluoride salts from the surface whereby a pore free boride coating of a desired depth is obtained in a shorter time by using a high current density. 15
6. A method of forming a boride coating on a low carbon steel workpiece which comprises:  
 forming an electric cell containing a molten fluoride electrolyte composed essentially of lithium fluoride, sodium fluoride and potassium fluoride and having said steel workpiece as the cathode joined through an external electrical circuit to a boron anode; 20  
 maintaining said electrolyte at a temperature of at least 900° C. in the absence of oxygen; 25  
 maintaining a current flowing in said electric cell so that the current density at the cathode will be greater than 4 amperes per square decimeter during the formation of the boride coating; and  
 stopping said current flow after a desired time duration of boriding is completed whereby a pore free boride coating of a desired depth is obtained in a shorter time by using a high current density. 30

## References Cited

## UNITED STATES PATENTS

3,024,176 3/1962 Cook ----- 204-39

TA-HSUNG TUNG, Primary Examiner

R. L. ANDREWS, Assistant Examiner